

## UNITED STATES PATENT OFFICE

1,922,993

NEW RESERVING PREPARATION AND  
RESERVE DYEING PROCESS

Gustav Torinus, Bad Soden on Taunus, Germany, assignor to General Aniline Works, Inc., New York, N. Y., a Corporation of Delaware

No Drawing. Application August 20, 1930,  
Serial No. 476,730, and in Germany September  
11, 1929

## 16 Claims. (Cl. 8—6)

The present invention relates to new reserving preparations and a process of reserving materials to be dyed with vat dyestuffs.

I have found that polyvinyl alcohols, especially when mixed with an oxidizing agent, such as, for instance, sodium meta-nitrobenzene sulfonate, sodium bichromate, or the like, are good agents for reserving materials which are to be dyed with vat dyestuffs. They are used, for instance, in the following manner: The material is printed with a paste containing a polyvinyl alcohol, water and an oxidizing agent, either alone or mixed with a substance having a mechanically reserving action, such as kaolin, drying the material and dyeing it in the usual manner in the warm dye liquor of a vat dyestuff. During this process the polyvinyl alcohols are precipitated, perhaps coagulated, by means of the alkalies present, particularly in the heat, and they, therefore, adhere to the parts of the material which have been printed and, in conjunction with the oxidizing agent incorporated in them, act as reserves and prevent access of the vat dyestuffs to the portions of the material to which the preparations are applied.

The present process may also be applied for producing colored reserves. In this case the reserve printing paste is mixed with, for instance, a diazo component and the material to be printed is impregnated with a coupling component.

The following examples serve to illustrate the invention, but they are not intended to limit it thereto:

35 *I. White-reserve-printing-preparation*

600 grams of an aqueous solution of polyvinyl alcohol of 25% strength are mixed with

40 200 grams of sodium meta-nitrobenzene sulfonate dissolved in

200 grams of water

1000 grams.

The preparation is printed on the material, dried and dyed at 75° C—80° C in the following vat, whereafter the material is washed and dried:

Dye-liquor

7 grams of N-dihydro-1.2-1'.2'-anthraqui-  
none azine powder

50 75 grams of glucose (1:1)

848 grams of boiling water

60 cc. of caustic soda solution of 40° Bé

10 grams of hydrosulfite concentrated powder

55 1 liter.

The material is dyed in this solution from 30 to 60 seconds.

*II. Red-reserve-printing-color*

|                                                                       |    |
|-----------------------------------------------------------------------|----|
| 600 grams of an aqueous solution of polyvinyl alcohol of 25% strength | 60 |
| 100 grams of sodium meta-nitrobenzene sulfonate                       |    |
| 100 cc. of the diazo solution of 5-chloro-2-aminotoluene              | 65 |
| 20 grams of crystallized acetate of sodium                            |    |
| 180 cc. of water                                                      |    |
| <hr/>                                                                 |    |
| 1000 grams.                                                           |    |

The red-reserve-printing-color is printed on material previously impregnated with the naphthol-preparation mentioned afterwards, dried intensely and dyed at 75° C—80° C in the liquor as indicated in Example 1, washed, soaped at boiling temperature, rinsed hot and dried. 75

*III. Orange-reserve-printing-color*

|                                                                        |    |
|------------------------------------------------------------------------|----|
| 600 grams of an aqueous solution of polyvinyl alcohol of 25% strength, | 80 |
| 100 grams of sodium meta-nitrobenzene sulfonate,                       |    |
| 100 cc. of the diazo solution of m-chloraniline,                       |    |
| 20 grams of crystallized sodium acetate,                               |    |
| 180 cc. of water                                                       | 85 |
| <hr/>                                                                  |    |
| 1000 grams.                                                            |    |

The material is printed and dyed as in Example II.

| Diazotized 5-chloro-2-aminotoluene         | 90  |
|--------------------------------------------|-----|
| 10 grams of 5-chloro-2-aminotoluene        |     |
| 20 grams of water                          |     |
| 11 cc. of hydrochloric acid of 20° Bé.     | 95  |
| 70 grams of ice and water                  |     |
| 4.2 grams of sodium nitrite are made up to |     |
| 110 cc.                                    | 100 |

## Naphthol-preparation:

|                                                                                        |     |
|----------------------------------------------------------------------------------------|-----|
| 20 grams of beta-hydroxynaphthoic acid-5-chloro-2-toluidide are made into a paste with |     |
| 20 grams of sodium Turkey red oil of 50% strength                                      | 105 |
| 30 cc. of caustic soda solution of 34° Bé are added and made up with hot water to      |     |
| <hr/>                                                                                  |     |
| 1 liter.                                                                               | 110 |

IV. *Pink-reserve-printing color*

40 grams of disulfuric acid ester of 4,4'-dimethyl-6,6'-dichloro-leuco-thioindigo

5 30 grams of ethylglycol

50 grams of sodium benzylsulfanilate

150 grams of kaolin

270 grams of water

10 400 grams of an aqueous solution of polyvinyl alcohol of 25% strength

30 grams of ammonium sulfocyanate

20 grams of sodium chlorate

10 grams of vanadate of ammonium of 1% strength

15 —

1000 grams.

This color is printed on the material, dried, steamed either for 10 minutes in a Mather-Platt or for 20 minutes in a steam vessel and dyed as in

20 Example I.

I claim:

1. The process which comprises printing material with a reserve printing paste comprising a polyvinyl alcohol and an oxidizing agent, drying the material thus treated and dyeing it in a vat in the usual manner.

2. The process which comprises printing material with a reserve printing paste comprising a polyvinyl alcohol, water and an oxidizing agent, drying the material thus treated and dyeing it in a vat in the usual manner.

3. The process which comprises printing material with a reserve printing paste comprising a polyvinyl alcohol, water, a substance of a mechanically reserving action and an oxidizing agent, drying the material thus treated and dyeing it in a vat in the usual manner.

4. The process which comprises printing material, impregnated with a coupling component, with a reserve printing paste comprising a polyvinyl alcohol, water, a diazo component and an oxidizing agent, drying the material thus treated and dyeing it in a vat in the usual manner.

5. The process which comprises printing material, impregnated with a coupling component, with a reserve printing paste containing a polyvinyl alcohol, water, a substance having a mechanically reserving action, a diazo component and an oxidizing agent, drying the material thus treated and dyeing it in a vat in the usual manner.

6. The process which comprises printing ma-

terial with a reserve printing paste comprising polyvinyl alcohol, water and sodium meta nitrobenzene sulfonate, drying the material thus treated and dyeing it in a vat in the usual manner.

7. The process which comprises printing material with a reserve printing paste comprising polyvinyl alcohol, water, kaolin and sodium meta-nitrobenzene sulfonate, drying the material thus treated and dyeing it in a vat in the usual manner.

8. The process which comprises printing material, impregnated with the 5-chloro-2-toluidide of the  $\beta$ -hydroxy naphthoic acid, with a reserve printing paste comprising polyvinyl alcohol, water, a diazotized 5-chloro-2-amino-toluene and sodium meta-nitrobenzene sulfonate, drying the material thus treated and dyeing it in a vat in the usual manner.

9. The process which comprises printing material, impregnated with the 5-chloro-2-toluidide of the  $\beta$ -hydroxynaphthoic acid with a reserve printing paste containing polyvinyl alcohol, water, kaolin, a diazotized 5-chloro-2-amino-toluene and sodium meta-nitrobenzene sulfonate, drying the material thus treated and dyeing it in a vat in the usual manner.

10. The process which comprises printing material with a reserve printing paste containing polyvinyl alcohol, water, sodium benzylsulfanilate, kaolin, sodium chlorate and the disulfonic acid ester of 4,4'-dimethyl-6,6'-dichloro-leuco-thioindigo, drying the material thus treated and dyeing it in a vat in the usual manner.

11. A new reserving preparation comprising polyvinyl alcohol and an oxidizing agent.

12. A new reserving preparation comprising polyvinyl alcohol, an oxidizing agent and a substance having a mechanically reserving action.

13. A new reserving preparation comprising, polyvinyl alcohol and sodium-meta-nitrobenzene sulfonate.

14. A new reserving preparation comprising polyvinyl alcohol, sodium meta-nitrobenzene sulfonate and kaolin.

15. A new reserving preparation comprising, polyvinyl alcohol and sodium benzylsulfanilate.

16. A new reserving preparation comprising, polyvinyl alcohol, sodium benzylsulfanilate and kaolin.

GUSTAV TORINUS. 125

55

130

60

135

65

140

70

145

75

150